

## UNITED STATES PATENT OFFICE

2,476,271

## LUBRICATING OIL ADDITIVE

John D. Bartleson, Cleveland, Ohio, assignor to  
The Standard Oil Company, Cleveland, Ohio, a  
corporation of Ohio

No Drawing. Application May 29, 1946,  
Serial No. 673,153

2 Claims. (Cl. 252—50)

1

This invention relates to lubricants containing anti-oxidant additives, suitable for use under various conditions under which lubricating oils or greases tend to deteriorate.

The objects achieved in accordance with the invention include the provision of lubricants or lubricating oils containing an anti-oxidant addition agent which inhibits the deposition of lacquer, the formation of acid and sludge, and the deterioration of other types which tend to occur under operating conditions. Other objects will be apparent as embodiments are described hereinafter.

In accordance with the invention, it has been found that an unsaturated tertiary aliphatic amine in which one of the aliphatic radicals is relatively long, i. e., contains at least 10 and generally not over 24 carbon atoms, and the other two radicals are relatively short, i. e., contain from 1 to 5 carbon atoms, inclusive, are particularly advantageous anti-oxidant additives for lubricants. A small amount of such an additive incorporated in a lubricating oil or grease imparts thereto a great improvement in its sludge, viscosity index, lacquer, and acid number characteristics.

Commercial octadecenylamine may be converted to corresponding dialkyl tertiary amine by heating with a lower alkyl chloride, e. g., methyl chloride. The reaction mass is treated with caustic and the tertiary amine recovered. It may be washed with water to remove inorganic salts, if desired. In view of its ready availability this amine will be used for illustrative purposes.

The amine used in accordance with the invention should contain at least one olefinic double bond in the molecule, preferably in the long chain. Typical unsaturated tertiary amines are: octadecenyl-dimethylamine, hexadecenyl-dimethylamine, tetradecenyl-dimethylamine, dodecenyl-dimethylamine, decenyl-dimethylamine, and the corresponding tertiary amines wherein either one or both of the methyl groups are replaced by ethyl, propyl, butyl or pentyl radicals, or the corresponding dienyl or trienyl amines. Analogous polyamines which contain no amine hydrogen, i. e., no hydrogen attached directly to a nitrogen are also suitable.

The amount of the additive to be incorporated in an oil or grease will depend on the characteristics of the base oil or grease and the intended

2

use. Some oils have more of a tendency to form acids, sludges and lacquer deposits than others, and such oils require larger quantities of the additive agent. In general, for lubricating oils the range is from 1 to 10% by weight but under some circumstances amounts as low as .01% show a significant improvement. For certain special uses the amount may be as high as 25.0% by weight. Of course, it will be uneconomical to add more of the additive than is necessary to impart the desired properties to the lubricant.

In order to demonstrate the properties of the unsaturated tertiary amines containing one long aliphatic chain as additives for lubricating oils, a number of amines were incorporated into a conventional lubricating oil. The lubricating oils containing these amines were tested according to laboratory test procedures for evaluating the service stability of oils as described in a paper by R. E. Burk, E. C. Hughes, W. E. Scovill and J. D. Bartleson presented at the Atlantic City meeting of the American Chemical Society in September 1941, and in another paper by the same authors presented at the New York city meeting of the American Chemical Society in September 1944, published in Industrial and Engineering Chemistry, Analytical Edition, vol. 17, No. 5, May 1945, pages 302-309. The latter paper also correlates the results of such laboratory tests with the so-called standardized "Chevrolet Engine Test."

Essentially the laboratory test equipment consists of a vertical thermostatically heated, large glass test tube, into which is placed a piece of steel tubing of about one-third its length and of much smaller diameter. A piece of copper-lead bearing strip is suspended within and from the upper end of the steel tube by a copper pin, and an air inlet is provided for admitting air into the lower end of the steel tube in such a way that in rising the air will cause the oil present to circulate. The test tube is filled with an amount of the oil to be tested which is at least sufficient to submerge the metals.

The ratios of surface active metals to the volume of oil in an internal combustion test engine are nearly quantitatively duplicated in the test equipment. In the "Standard" test the temperature used is approximately the average temperature of the crankcase. The rate of air flow per

volume of oil is adjusted to the same as the average for a test engine in operation. Of the catalytic effects, those due to iron are the most important. They are empirically duplicated by the addition of a soluble iron salt. Those due to lead-bromide are duplicated by its addition. In the "Standard" test, 0.012% of iron salt is added; and in the "Iron Tolerance" test this is increased to 0.05%. The duration of the test is adjusted to that usually used in engine type tests. The "Iron Tolerance" tests were run at 280° F. for thirty-six hours.

As is shown by the data in the paper referred to, the laboratory tests have been correlated with engine tests and the properties of the oil in an engine may be determined from the result of the laboratory tests.

The results given in the following table were obtained from tests using:

A 160 cubic centimeter sample of the lubricant 20 composition  
70 liters of air per hour  
100 square centimeters of steel surface  
4.4 square centimeters of copper-lead surface  
1.0 square centimeters of copper surface  
0.01% by weight of lead bromide powder  
0.05% soluble iron calculated as  $Fe_2O_3$   
(Ferric 2-ethyl hexoate in C. P. benzene)

The lacquer is deposited on the steel tube and is determined by difference in weight of the tube after washing with chloroform and drying to constant weight. The used oil was sufficient to enable the determination of all of the usual oil tests, viz. sludge (isopentane insolubles), viscosity, acid number, etc.

The data in the following table shows the results obtained in testing the new compositions by the tests described.

"Standard" tests were carried out on a conventional Mid-Continent acid-treated lubricating oil (SAE 30) and the same oil containing 3% of octadecenyl-dimethylamine. The results are as follows:

|                                                      |      |      |
|------------------------------------------------------|------|------|
| Concentration of additive in per cent by weight..... | None | 3    |
| Lacquer (mgs.).....                                  | 21.9 | 1.6  |
| Sludge (mgs.).....                                   | 532  | 20.3 |
| Acid No.....                                         | 6.6  | 1.2  |
| Viscosity increase.....                              | 635  | 61   |

The unsaturated tertiary amine improves every indicated characteristic of the oil.

"Iron Tolerance" tests on a conventional Mid-Continent acid-treated lubricating oil base stock (SAE 30) containing different amine compositions were run. The results given in the following table are representative.

The amine compositions used for comparative purposes are:

*Example 1.*—Composition comprising primarily octadecenyl-dimethylamine (unsaturated tertiary)

*Example 2.*—Composition comprising primarily octadecylamine (primary saturated)

*Example 3.*—Composition comprising primarily octadecenylamine and octadecadienylamine (primary unsaturated)

*Example 4.*—Composition comprising primarily dioctadecylamine (secondary saturated)

*Example 5.*—Composition comprising primarily cetyl dimethylamine (tertiary saturated)

The amounts of these amines used in the tests

are calculated to give approximately equal nitrogen concentrations.

Table

| Additive of Example No.....                          | None | 1   | 2   | 3   | 4    | 5    |
|------------------------------------------------------|------|-----|-----|-----|------|------|
| Concentration of Additive in per cent by weight..... | None | 1.5 | 1.5 | 1.5 | 3.0  | 1.38 |
| Sludge (isopentane insoluble in milligrams).....     | 809  | 365 | 420 | 692 | 663  | 484  |
| Acid Number.....                                     | 9.4  | 3.7 | 6.6 | 7.8 | 10.3 | 7.5  |
| Viscosity Increase (SUS).....                        | 658  | 238 | 416 | 718 | 1405 | 765  |

It will be evident from this data that the unsaturated tertiary amine of Example 1 is markedly superior to the saturated primary amine of Example 2, the primary unsaturated amine of Example 3, the saturated secondary amine of Example 4, or the saturated tertiary amine of Example 5. A comparison of Examples 1 and 3 shows the effect of replacing the two hydrogens to form an unsaturated tertiary amine, and a comparison of Examples 1 and 4 shows the improvement attributable to the double bond, i. e., decreased sludge, lower acid number (indicating less corrosion), and lower viscosity increase, thereby indicating improved antioxidant effects for the unsaturated tertiary amine. The additives will find particular use in specialty oils, such as turbine, instrument, anti-rust oils, etc.

The expression "deteriorative lubricant" refers to any oils and greases which are subject to oxidation, especially these from petroleum sources.

The invention broadly contemplates all variations and modifications which will be apparent to one skilled in the art in view of the foregoing disclosures, except as do not come within the scope of the appended claims.

I claim:

1. A lubricant consisting essentially of a mineral lubricating oil and an amount to inhibit oxidation of said oil of an oxidation inhibiting amine having the formula



wherein R is an aliphatic hydrocarbon radical of 10 to 24 carbon atoms and having one double bond, and R<sub>1</sub> and R<sub>2</sub> are alkyl radicals having one to five carbon atoms.

2. A lubricant comprising a mineral lubricating oil and an amount to inhibit oxidation of said oil of an oxidation inhibiting amine having the formula



where R is an aliphatic hydrocarbon radical of 18 carbon atoms and having one double bond, and R<sub>1</sub> and R<sub>2</sub> are methyl groups.

JOHN D. BARTLESON.

#### REFERENCES CITED

The following references are of record in the file of this patent:

#### UNITED STATES PATENTS

| Number    | Name           | Date          |
|-----------|----------------|---------------|
| 1,888,023 | Adams          | Nov. 15, 1932 |
| 2,110,199 | Carothers      | Mar. 8, 1938  |
| 2,268,608 | McNulty et al. | Jan. 6, 1942  |